

# UNITED STATES PATENT OFFICE

GEORGE SPRUNG, OF VANCOUVER, BRITISH COLUMBIA, CANADA.

## ROAD-MAKING MATERIAL.

1,091,777.

Specification of Letters Patent. Patented Mar. 31, 1914.

No Drawing.

Application filed October 4, 1913. Serial No. 793,332.

To all whom it may concern:

Be it known that I, GEORGE SPRUNG, a citizen of the Dominion of Canada, residing at Vancouver, in the Province of British Columbia, Canada, have invented certain new and useful Improvements in Road-Making Material, of which the following is a specification.

This invention relates to an improved road construction which is particularly designed to form a simple and comparatively inexpensive roadway, the surface of which will not be impaired by ordinary auto traffic and that will be elastic and dustless.

15 The invention is particularly described in the following specification.

The essential principle of the invention lies in the application to an ordinary Macadam or rock roadway of a novel bonding material that will compactly fill all the interstices of the rock when the same is rolled. This bonding material is a mixture of sawdust with a sufficient amount of a bituminous material such as heavy road oil (crude oil) or asphaltum or tar as will effectively cover the surfaces of the rock, permeate the material of the sawdust and that will fill the interstices of the same. The oil, asphaltum, or tar, is used as a strong adherent material holding the interlocked particles of sawdust together, and is not merely a medium in which a certain proportion of sawdust is embodied. If the oil is in excess it does not hold the particles together but serves as a lubricant permitting them to slide past one another under the rolling action of the traffic. The same principle should prevail in the association of the bonding material of sawdust and oil with the rock. The pieces of rock are not merely associated in a composition with oil and sawdust but the rock must be strongly rolled together so as to have a minimum of interspace, and these interspaces must be filled with tightly packed sawdust bound together with asphaltum material.

All road oils carry a large proportion of asphaltum or the like and while the more volatile and soluble oils may evaporate, or be washed out, sufficient of the heavier insoluble parts remain to bind the sawdust together.

55 The preferred method of applying this bonding material is to take the rock (broken to the size as for an ordinary Macadam

road) and such proportion of sawdust as will compactly fill the interspaces of the rock when the roadway has been heavily rolled with as much of any heavy road oil, asphaltum or tar as will cover the surfaces of the pieces of rock, permeate the sawdust and fill the interstices of the same when it is tightly packed together. These proportions will vary according to the character of the road required, the nature of the rock and of the sawdust. These materials, in such proportion as will satisfy the above requirements, are thoroughly mixed together and are spread upon the road, and the road is heavily rolled. The result is a compact elastic road bed, the wearing surface of which is the rock and the bonding material is the tightly packed, elastic, asphaltum-cemented sawdust. The same result may be obtained, although not so effectively, by spreading the rock, as in making an ordinary Macadam road; thereafter spreading sawdust over the rock and scarifying it to insure that the sawdust works into the wide interstices of it. After the sawdust is thoroughly worked among the rock, the heavy oil, asphaltum or tar is spread over the rock and sawdust in sufficient quantity to permeate the sawdust filling between the interstices, of the rock, and the road surface is then heavily rolled to pack the rock tightly together and to compress the sawdust within its interstices.

90 It must be distinctly understood that the sawdust is not designed to give substance or body to a bonding material of asphaltum or other composition of matter, but the heavy oil is added to bind together the closely compressed sawdust.

It will, in all likelihood, be found advisable to apply a top dressing of sand or fine rock crushings to the surface of the road bed when it is turned over for use, but this will not form a constituent part of the road, but is merely applied to prevent the asphaltum material from sticking to the wheels of passing vehicles and possibly lifting the road surface.

Having now particularly described my invention, I hereby declare that what I claim as new and desire to be protected in by Letters Patent, is:

110 1. A road making material, comprising broken rock and a filling for the interstices of the closely packed rock said filling com-

prising sawdust permeated with a bituminous material.

2. A road making material, comprising broken rock with sufficient sawdust soaked with a bituminous material, to fill compactly the interstices between the rock when the same has been heavily rolled.

In testimony whereof I affix my signature in presence of two witnesses.

GEORGE SPRUNG.

Witnesses:

ROWLAND BRITTAINE,  
MAY WHYTE.